# EUROPEAN PATENT SPECIFICATION

(11) **EP 2 255 937 B1**
(45) Date of publication and mention of the grant of the patent: **03.06.2015**
(21) Application number: 09172995.4
(22) Date of filing: 14.10.2009
(51) Int. Cl.: B27M 1/02, B27M 3/04

(54) **Manufacturing method for a surface-strengthened solid wood floor board**
Herstellungsverfahren für einen oberflächenverstärkten Massivholzbodenbelag
Procédé de fabrication de plancher en bois massif renforcé en surface

(30) Priority: 29.05.2009 CN 200910099265
(43) Date of publication of application: 01.12.2010
(73) Proprietor: Zhejiang Shiyou Timber Co. Ltd., Huzhou City, Zhejiang 313009 (CN); Tu, Dengyun, Huzhou City, Zhejiang 313009 (CN)
(72) Inventor: Tu, Dengyun, Huzhou City, Zhejiang 313009 (CN); Ni, Yuezhong, Huzhou City, Zhejiang 313009 (CN)
(74) Representative: Elzaburu Marquez, Alberto

(56) References cited:
- WO-A1-01/68332
- WO-A1-2009/094792
- GB-A- 861 347
- US-A- 3 292 676
- US-A- 3 591 448
- US-A- 5 992 043
- US-A1- 2008 263 890
- DATABASE WPI Week 200843 Thomson Scientific, London, GB; AN 2008-G72470 XP002599893 & CN 101 007 415 A (UNIV ZHEJIANG FOREST) 1 August 2007 (2007-08-01)
- DATABASE WPI Week 199826 Thomson Scientific, London, GB; AN 1998-290773 XP002599894 & JP 10 100108 A (NODA KK) 21 April 1998 (1998-04-21)

## Description

### Field of Invention

The present invention relates to the technical field of wood processing, in particular to a manufacturing method for a surface-strengthened solid wood floor board

### Related Art

The hardwood products are popular for most consumers, especially the hardwood furniture and flooring. However, because of the slowly growing hardwood trees, the difficulty to obtain required amount of woods in short term, the forest protection, and the tree-felling ban in many countries, leading to the shortage of raw materials, it is difficult for those hardwood furniture plants and flooring plants to provide sufficient hardwood products for the consumers. Under the situation of the continuously decreasing natural forest resources and the wood supply almost depending upon the fast-growing and high-yielding artificial production forest, the current research focuses on the solution of improving the mechanical strength and processability of the woods obtained from the artificial forest by means of the densification processing method so as to substitute the hardwoods.

The Chinese patent application, whose publication number is CN1282654A, discloses a patent technology titled "An Manufacturing Method for Reinforced Solid Wood Floor Board of Composite Tongue-and-groove Type" by Mr. Yang Zhiliang, **characterized in that** the board core is made from pine wood or fast-growing forest wood, surface layer thereof is affixed to a wood-grain decorative layer and an aluminum oxide (Al₂O₃) wearable layer, as well as a melamine fire-retardant layer, periphery thereof is tongued-and-grooved to produce flooring. The produced flooring by means of this technology is of multi-layer composite type without more intense pressure and more glue applied, so the strength of such flooring is just at normal level. Furthermore, another Chinese patent, whose publication number is CN1195611C, discloses a patent technology titled "Preparing Method for Base Materials of Reinforced Wood Floor Board" by the Wuhan Rongde Industry Co., Ltd. The sawdust is used as the raw material which is glued and pressed into the base material of flooring. Although the technology makes use of the wood waste, the mechanical strength of it is worse than the log fiber when the sawdust is used as raw material. Therefore, it can be seen that all these two patents provide low-strength flooring, but such flooring are not popular for most consumers who prefer solid wood products.

As most properties of the solid wood profiles, such as hardness, wear resistance, bending strength and dimension stability, are mostly dependent upon the surface, the surface of the timber is densified to a certain depth to increase the density and harden the surface. After the densification, interior density of the timber would not change or would be increased slightly, but the physical and mechanical properties of the timber would be improved, leading to saved cost and decreased loss of timber volume. Therefore, the densification is an ideal method for improving the properties of the soft timber obtained from the artificial forest.

There are also other available technologies which can improve the density and hardness of the timber surface. Technical solution for these technologies is as follows, making organics, such as organic resin, and inorganic metallic elements permeate through the timber's surface layer to a certain depth so as to densify the timber surface. The phenolic resin, urea-formaldehyde resin, modified melamine resin, isocyanate resin, etc. may cross linked with the timber to improve hardness of the timber surface, but such densified timber is greatly pollution hazardous.

Someone even further compresses the resin-impregnated timber to a certain degree, acquiring higher degree of densification. Furthermore, the resin can better fix the compressive deformation. But there are still some shortcomings such as pollution and process complexity.

Currently, the method for densifying the timber by hot pressing has been reported, for example, the Chinese patent by the Zhejiang Forestry University, whose publication number is CN101007415A, discloses a manufacturing process for surface-strengthened flooring, it consisting of (1) a step of primarily processing raw materials, in which Chinese fir wood or the like, that is a thinning wood of the fast-growing forest, pine wood and aspen wood, as well as the logs with oven-dry density less than 600kg/m³ are processed into coarse boards; (2) a step of drying, in which the coarse boards are dried based on the available drying schedule, controlling the final water content within 4%-10%, preferably within 5%-8%; (3) a step of rough planning, in which four sides of the coarse boards are roughly planed using the quadrilateral planing machine; (4) a step of heating, in which the coarse boards are heated in the drying kiln to the temperature of 100-150° C for 10-60 minutes; (5) a step of resin dipping, in which the coarse boards are thrown into the normal-temperature resin pool immediately after being taken out from the drying kiln by means of hot and cold dipping method to dip the board for 2-25 minutes, wherein the solid content is 20%-40% and the thermosetting resins, such as phenolic resin or urea-formaldehyde resin are used; (6) a step of hot pressing, in which the board materials are hot pressed using the normal multilayer thermal press or the continuous thermal press, with the ratio of compression controlled within 5%-20%, the temperature within 100-190°C and the time of hot pressing within 200-2800s; wherein the time of hot pressing changes correspondingly with different woods, different resins and temperatures; (7) a step of aging, in which the hot pressed board materials are aged for 4-48h at the normal temperature so as to eliminate the internal stress and stabilize the dimension; (8) a step of fine machining, in which the final products for consumers are obtained by planing, sharpening, sand grinding and painting. The surface strength of the board obtained using the above-mentioned method is higher. To achieve an ideal surface densification effect when radially or chordwisely compressing the board along the cross striation, however, the following conditions shall be satisfied firstly, high temperature and humidity and sufficient softening of the surface layer of the board, low temperature and non-softening of partial intermediate layer, at the same time to control the low ratio of compression or compression rate. The possibility of non-compressed under higher compression rate even the intermediate layer has not been softened is little, in particular when radially compressing the board, it is easy to compress and deform the spring wood cell as the cell wall is thin. Therefore, the process method of densifying the surface layer of the board through compression requires high temperature but short time. To avoid the compression failure of the surface layer after the compression, normally the hot pressed board shall be impregnated into the resin for a period. In addition, the board shall be surface grooved, before the hot pressing, and then put into the water to improve the moisture content of the board. Therefore, the process is comparatively complicated and not environmentally friendly.

US 3591448 A, which is considered to be the closest prior art document and refers to "Wood with a densified surface layer and method of making same", relates to a method of densifying the surface of natural wood which consists of the steps of:
- selecting wood having a substantial difference in the density of the spring wood and the summer wood and whose moisture content is above about 6%,
- heating a flat plate to a temperature above about 121 degrees C (250 degrees F),
- inserting the heated plate between the wood and a cold press platen,
- quickly applying pressure on the wood and increasing the pressure rapidly while heat passes from the plate into the wood until the spring wood collapses,
- maintaining pressure on the wood during the time interval in which the heat continues to flow into the wood, the maximum temperature has been reached, the direction of the heat flow is reversed, and the temperature of the crushed wood fibers has fallen well below 100 degrees C (212 degrees F),
- then releasing the pressure and removing the wood from the press.

### SUMMARY OF THE INVENTION

An object of the present invention is to provide a method for manufacturing a surface-strengthened solid wood floor board. The method is convenient, simple and environmentally friendly, which solves the technical problems of being complicated and severe pollution of the available processes.

The said technical objects are achieved by a manufacturing method according to claim 1.

The present invention is suitable for a variety of woods, such as Chinese fir wood, pine wood, cotton wood, Manchuran-tree wood, paulownia wood, birch wood and basswood. These woods can all be processed using the said method.

As the moisture content differs for different woods, the log profiles are to be dried first. The moisture content of the dried log profiles are controlled within 7-16%, more preferably within 7-13%. If moisture content is too low, the possibility of log profiles being fractured is substantially increased due to the compression in the subsequent stage, and also the rebound degree after the compression is strengthened. It is shown by test that if the moisture content is excessively high, and then uniform moisture distribution is created inside the wood, the wood easily deforms after the compression, meanwhile, the interior will crack, even the surface. In addition, dimension of the wood decreases due to drop of the moisture inside the wood after the compression, leading to difficulty to acquire compressed wood with required dimension:
As a preference of the above-mentioned technical solution, the moisture content of the log profiles after drying are controlled within 8-10%, preferably within 8-9%. As another preference, the moisture content of the log profiles after drying are controlled within 10-14%, preferably within 10-12%.

As a preference for the present invention, the surfaces of the log profiles dried are to be polished. If the surface is not polished, the compression will be non-uniform due to the protuberances on the wood profiles, leading to insufficiently level surface of the compressed part after the partial recovery. Furthermore, compression of the protuberances may greatly damage texture of the wood profiles resulting in decrease of the mechanical properties of the wood profiles. Meanwhile, the said polishing can make the hot press quickly heat the log profiles so as to realize fast compression.

Temperature of the log profiles in the hot press is very crucial, and temperature of the said hot press is the temperature of the pressing plate of the hot press. It is shown by test that the higher the hot pressing temperature, under certain conditions within hot pressing time, the smaller the rebounded rate of the compression of the profiles. Take the cryptomeria for example, it will be compressed for 7 days, the recovery rate of compression thereof, when the hot pressing temperature is 60°C, is 83%, while the recovery rate of compression thereof, when the hot pressing temperature is 100°C, is 58%. So controlling the hot pressing temperature for the present invention can achieve suitable recovery rate of compression. Excessively high hot pressing temperature largely affects the mechanical properties of the wood profiles, as degradation of the wood fiber, under over-high temperature, becomes severe. Furthermore, over-high hot pressing temperature makes it difficult to realize the cross link among fibers, leading to largely decreased mechanical properties of the profiles. As the preference of the above-mentioned scheme, the temperature of the hot press is kept within 220°C-250°C. The optimum scheme is to keep the temperature within 230°C-250°C.

As the preference of the present invention, the compression rates of the said log profiles are controlled within 15%-25% when being compressed, preferably within 16%-20%. Over-high compression rate results in over-long compression time and overweight profiles, meanwhile severely affects the recovery rate of compression and mechanical properties of the profiles. Over-low compression rate dissatisfies the requirements for surface mechanical properties. Meanwhile the interior of the profiles may swell once the water penetrates through the surface layer in a humid environment, since over-low compression rate results in thinner surface-strengthened layer that provides weak obstruction to the outer environment. As the preference of the above-mentioned solution, the said compression rate is controlled within 17-23%.

To better control the recovery rate of compression, the said log profiles that has been compressed needs to be kept warm for a certain period. Also, over-long warm-keeping period may damage the mechanical properties of the profiles. Temperature for the said warm-keeping may be same with the hot pressing temperature, or 10°C-80°C lower than the hot pressing temperature, which almost does not affect properties of the profiles. Period for the said warm-keeping is preferably within 20-40 minutes. The said warm-keeping shall be generally conducted under the condition that the wood profiles is subject to the applied stress from the hot pres.

Under the temperature of 210°C-220°C, the warm-keeping effect is better if the warm-keeping period is within 50-60 minutes, and the compressed profiles has higher dimension stability, color of the surface thereof is not dark.

As a further preference of the present invention, the said warm-keeping lasts for 20-40 minutes. As another preference of the present invention, the said warm-keeping lasts for 35-40 minutes. These two different solutions differ in the color and the dimension stability of the compressed profiles.

When the log profiles are compressed, the compressing speed obviously affects the properties of the profiles other than the hot pressing temperature and compression rate. In one embodiment, the said speed at which the hot press compresses log profiles is within 4mm/s-10mm/s, the surface strength of the profiles improves greatly. One further preferable embodiment is to control the compressing speed of the hot press within 4mm/s-6mm/s, another still preferable embodiment is to control the compressing speed of the hot press within 8mm/s-9mm/s, and the most preferable embodiment is to control the compressing speed of the hot press within 7mm/s-8mm/s.

Another important factor to obtain the said profiles of the present invention is the moisture content of the profiles. Inside the profiles, there are a number of pores, which provides the profiles with water-absorption function. Once the moisture content is suitable and the exterior of the profiles is sealed, the profiles can adapt for largely changing humidity environment, having no water absorbed or dehydrated. After the warm-keeping, the moisture content of the profiles is adjusted to 6-9%, ensuring that the profiles does not deform even after long-term use in diversified climate conditions. The method for controlling the moisture content after the warm-keeping and cooling is diversified, for example, controlling the moisture content in the balance room where the temperature and humidity are adjustable, the drying kiln or under atmospheric conditions.

As preference of the present invention, the moisture contents of the profiles are adjusted to 6-7% after the warm-keeping. As another preference of the above-mentioned embodiment, the moisture content of the profiles is adjusted to 7-8% after the warm-keeping.

As preference of the present invention, control of the said moisture content is realized by placing the log profiles, which has been cooled, in the moisture control room, the temperature thereof is 40°C-65°C, the relative humidity of it is 75%-95%. After the moisture content of the profiles achieves the required level, it will be taken out from the moisture control room. Over-high temperature results in rebound of the compressed part of the surface layer, instead of strengthening the surface, while over-low temperature results in excessively long term placing and thereby affects the production efficiency.

The present invention uses high temperature so as to dry the wood in a high-temperature and compression condition. In addition, the high temperature degrades the hydrophilic group in the process of the hemicellulose and lignin degradation and greatly decreases the hygroscopicity of the wood. These two actions fix the compression of the surface layer of the wood so as to eliminate the rebound of the surface compression.

The profiles of the present invention can be further processed according to demand after the step of controlling of the moisture content is finished. For example, if the profiles are to be manufactured into solid wood floor board, it is required to tongue and groove the profiles and later to conduct the surface sanding and finishing. Such solid wood floor board, the recovery rate of compression thereof is low and the hardness of the paint film is high, can be used in most climate conditions, and can be widely used in humid and dry conditions. No keel and nailing are required when installing such floor board, which greatly reduces the installation cost and the damages to the houses. Meanwhile the comparatively simple process reduces the manufacture cost and generates low pollution.

Surface strengthened solid wood floor boards are manufactured, wherein the density of it is 300-580Kg/m³, thickness of the reinforced surface is 1-5mm, hardness of the paint film on the reinforced surface is 2H-8H and overall moisture content of the profiles is 6-9%.

The said solid wood floor boards contain no impurities of organic resin and inorganic metal elements, which is of "pure" solid wood type and almost pollution-free. The overall density of it is low and the hardness of the paint film of the reinforced surface is relatively high.

Log for the said surface reinforced solid wood floor boards are relatively soft, such as pine wood, Chinese fir wood, cottonwood and paulownia wood. Normally, density of the log is 250-480Kg/m³, which is not ideal for the manufacture of the flooring requiring high hardness. The said floor boards have higher hardness of the paint film on the strengthened surface, more stable overall moisture content compared with other solid wood floor boards with same density, therefore, they are more suitable for the wider range of climate conditions.

Preferably, the present invention is made using the log with smaller density, about 250-420Kg/m³, so the surface reinforced solid wood profiles with smaller density of 300-500Kg/m³ can be made.

### DETAILED DESCRIPTION OF THE INVENTION

This embodiment only explains the present invention, but not limits the present invention. The person skilled in the field can make modifications that have no creative contribution on this embodiment according to demands after reading this Description, and these modifications are protected by the patent law if they are within the scope of the claims of the present invention.

Example 1: a method for manufacturing the surface reinforced solid wood flooring uses Populus ussuriensis as the log. It comprises the steps of cutting the dried wood in a reasonable way according to the size of the solid wood to be manufactured to obtain a certain batch of same-sized sawed woods so as to perform subsequent drying and processing. The Populus ussuriensis wood is subsequently cut into blocks and they can be stacked, and then heavy object is put on the top of the stack, conveying the stack by fork into the drying kiln for drying, which is steam-heating head wind type, and controlling the moisture content at about 8%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 25mm thick polished wood profiles into the hydraulic three-layer hot press, make the hot pressing plate of the said hot press face the surface to be strengthened, adjust the temperature of the said hot pressing plate to 220°C, control the pressing speed of the hot pressing plate to 4mm/s, press the wood profiles being compressed in the hot press to 21mm thickness, pressure of the hot press when pressing is 25MPa. After finishing the pressing, maintain pressure and keep warm the wood profiles for 40 minutes, 40 minutes later slowly release the pressure by controlling the releasing speed to 0.01mm/s, place the wood profiles indoors for natural cooling. Put the cooled profiles in the moisture control room for four days, the relative humidity thereof is around 90% and the temperature thereof is 50°C. After controlling the moisture, the moisture content is within 6-7%. Store the profiles for a certain period, after which perform tongue-and-groove, surface sanding and surface finishing to acquire a solid wood floor board. Hardness of the 2-3mm thick upper part of the compressed surface of the floor board of the present invention is obviously strengthened, and moisture content of the floor board obtained in this embodiment is within 6-7%, which stays stable in all climate conditions. Density of the said solid wood floor board is 466kg/m³, and hardness of the paint film of the strengthened surface is 5-6H. Two sides of the solid wood flooring in this embodiment are tongued-and-grooved, the upper surface thereof is the strengthened surface, and thickness, of the strengthened layer is H = 2-3mm, the lower surface of the solid wood floor board is not strengthened, which not only saves the wood but also prevents the lower surface from swelling due to wetting. Chamfers of the strengthened layer of the solid wood floor board are coated with the seal paint, which penetrates through the interior of the strengthened layer, thereby effectively preventing the chamfers from absorbing water and consequently avoiding swelling.

Example 2: a method for manufacturing the surface reinforced solid wood flooring uses paulownia as the log. It comprises the steps of cutting the dried wood in a reasonable way according to the size of the solid wood to be manufactured to obtain a certain batch of same-sized sawed woods so as to perform subsequent drying and processing. The cut paulownia wood is formed into blocks and they can be stacked, and then heavy object is put on the top of the stack, conveying the stack by fork into the drying kiln for drying, which is steam-heating head wind type, and controlling the moisture content at about 7%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 30mm thick polished wood profiles into the hydraulic three-layer hot press, make the hot pressing plate of the said hot press face the surface to be strengthened, adjust the temperature of the said hot pressing plate to 250°C, control the pressing speed of the hot pressing plate to 10mm/s, press the wood profiles being compressed in the hot press to 24mm thickness, pressure of the hot press when pressing is 20MPa. After finishing the pressing, maintain pressure and keep warm the wood profiles for 20 minutes, 20 minutes later slowly release the pressure by controlling the releasing speed to 0.01 mm/s, place the wood profiles indoors for natural cooling. Put the cooled profiles in the moisture control room for six days, the relative humidity thereof is around 85% and the temperature thereof is 50°C. After controlling the moisture , the moisture content is within 7-8%. Store the profiles for a certain period, after which perform tongue-and-groove, surface sanding and surface finishing to acquire a solid wood floor board. Hardness of the 3-4mm thick upper part of the compressed surface of the floor board of the present invention is obviously strengthened, and moisture content of the flooring obtained in this embodiment is within 7-8%, which stays stable in all climate conditions. Density of the said solid wood floor board is 350kg/m³, and hardness of the paint film of the strengthened surface is 2-3H.

Example 3: a method for manufacturing the surface reinforced solid wood flooring uses basswood as the log. It comprises the steps of cutting the dried wood in a reasonable way according to the size of the solid wood to be manufactured to obtain a certain batch of same-sized sawed woods so as to perform subsequent drying and processing. The cut basswood wood is formed into blocks and they can be stacked, and then heavy object is put on the top of the stack, conveying the stack by fork into the drying kiln for drying, which is steam-heating head wind type, and controlling the moisture content at about 12%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 25mm thick polished wood profiles into the hydraulic three-layer hot press, make the hot pressing plate of the said hot press face the surface to be strengthened, adjust the temperature of the said hot pressing plate to 210°C, control the pressing speed of the hot pressing plate to 6mm/s, press the wood profiles being compressed in the hot press to 21mm thickness, pressure of the hot press when pressing is 20MPa. After finishing the pressing, maintain pressure and keep warm the wood profiles for 60 minutes, 60 minutes later slowly release the pressure by controlling the releasing speed to 0.1mm/s, place the wood profiles indoors for natural cooling. Put the cooled profiles in the moisture control room for eight days, the relative humidity thereof is around 85% and the temperature thereof is 55°C. After controlling the moisture, the moisture content is within 8-9%. Store the profiles for a certain period, after which perform tongue-and-groove, surface sanding and surface finishing to acquire a solid wood flooring. Hardness of the 2.5-3mm thick upper part of the compressed surface of the floor board of the present invention is obviously strengthened, and moisture content of the floor board obtained in this embodiment is within 8-9%, which stays stable in all climate conditions. Density of the said solid wood flooring is 422kg/m³, and hardness of the paint film of the strengthened surface is 3-4H.

Example 4: a method for manufacturing the surface reinforced solid wood flooring uses Populus ussuriensis as the log. It comprises the steps of cutting the dried wood in a reasonable way according to the size of the solid wood to be manufactured to obtain a certain batch of same-sized sawed woods so as to perform subsequent drying and processing. The cut Populus ussuriensis wood is formed into blocks and they can be stacked, and then heavy object is put on the top of the stack, conveying the stack by fork into the drying kiln for drying, which is steam-heating head wind type, and controlling the moisture content at about 12%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 28mm thick polished wood profiles into the hydraulic three-layer hot press, make the hot pressing plate of the said hot press face the surface to be strengthened, adjust the temperature of the said hot pressing plate to 230°C, control the pressing speed of the hot pressing plate to 8mm/s, press the wood profiles being compressed in the hot press to 23mm thickness, pressure of the hot press when pressing is 25MPa. After finishing the pressing, maintain pressure and keep warm the wood profiles for 35 minutes, 35 minutes later slowly release the pressure by controlling the releasing speed to 0.01mm/s, place the wood profiles indoors for natural cooling. Put the cooled profiles in the moisture control room for four days, the relative humidity thereof is around 95% and the temperature thereof is 55°C. After controlling the moisture, the moisture content is within 8-9%. Store the profiles for a certain period, after which perform tongue-and-groove, surface sanding and surface finishing to acquire a solid wood floor board. Hardness of the 3-5mm thick upper part of the compressed surface of the floor board of the present invention is obviously strengthened, and moisture content of the floor board obtained in this embodiment is within 8-9%, which stays stable in all climate conditions. Density of the said solid wood flooring is 477kg/m³, and hardness of the paint film of the strengthened surface is 6-8H.

Example 5: a method for manufacturing the surface reinforced solid wood flooring uses Populus ussuriensis as the log. It comprises the steps of cutting the dried wood in a reasonable way according to the size of the solid wood to be manufactured to obtain a certain batch of same-sized sawed woods so as to perform subsequent drying and processing. The cut Populus ussuriensis wood is formed into blocks and they can be stacked, and then heavy object is put on the top of the stack, conveying the stack by fork into the drying kiln for drying, which is steam-heating head wind type, and controlling the moisture content at about 10%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 27mm thick polished wood profiles into the hydraulic three-layer hot press, make the hot pressing plate of the said hot press face the surface to be strengthened, adjust the temperature of the said hot pressing plate to 240°C, control the pressing speed of the hot pressing plate to 6mm/s, press the wood profiles being compressed in the hot press to 23mm thickness, pressure of the hot press when pressing is 25MPa. After finishing the pressing, maintain pressure and keep warm the wood profiles for 35 minutes, 35 minutes later slowly release the pressure by controlling the releasing speed to 0.01mm/s, place the wood profiles indoors for natural cooling. Put the cooled profiles in the moisture control room for five days, the relative humidity thereof is around 85% and the temperature thereof is 65°C. After controlling the moisture, the moisture content is within 6-7%. Store the profiles for a certain period, after which perform tongue-and-groove, surface sanding and surface finishing to acquire a solid wood flooring. Hardness of the 2-3mm thick upper part of the compressed surface of the floor board of the present invention is obviously strengthened, and moisture content of the floor board obtained in this embodiment is within 7-8%, which stays stable in all climate conditions. Density of the said solid wood floor board is 460kg/m³, and hardness of the paint film of the strengthened surface is 2-3H.

Example 6: a method for manufacturing the surface reinforced solid wood flooring uses Populus ussuriensis as the log. It comprises the steps of cutting the dried wood in a reasonable way according to the size of the solid wood to be manufactured to obtain a certain batch of same-sized sawed woods so as to perform subsequent drying and processing. The cut Populus ussuriensis wood is formed into blocks and they can be stacked, and then heavy object is put on the top of the stack, conveying the stack by fork into the drying kiln for drying, which is steam-heating head wind type, and controlling the moisture content at about 9%. Polish surface of the block-shaped wood that has been dried with WEINIG four-side planer (manufactured by the German WEINIG GROUP, mode: U23 EL), select one of the polished surfaces as the surface to be strengthened, make the selected polished surface parallel to the fiber direction of the wood, put the 27mm thick polished wood profiles into the hydraulic three-layer hot press, make the hot pressing plate of the said hot press face the surface to be strengthened, adjust the temperature of the said hot pressing plate to 225°C, control the pressing speed of the hot pressing plate to 9mm/s, press the wood profiles being compressed in the hot press to 22mm thickness, pressure of the hot press when pressing is 25MPa. After finishing the pressing, maintain pressure and keep warm the wood profiles for 45 minutes, 45 minutes later slowly release the pressure by controlling the releasing speed to 0.01mm/s, place the wood profiles indoors for natural cooling. Put the cooled profiles in the moisture control room for four days, the relative humidity thereof is around 95% and the temperature thereof is 65°C. After controlling the moisture, the moisture content is within 7-8%. Store the profiles for a certain period, after which perform tongue-and-groove, surface sanding and surface finishing to acquire a solid wood floor board. Hardness of the 2-3mm thick upper part of the compressed surface of the floor board of the present invention is obviously strengthened, and moisture content of the floor board obtained in this embodiment is within 7-8%, which stays stable in all climate conditions. Density of the said solid wood flooring is 468kg/m³, and hardness of the paint film of the strengthened surface is 2-3H.

In the present invention, the moisture content of the wood uncompressed is determined according to the GB 1931-91 Method for determination of the moisture content of wood. The moisture content of the finished floor board is determined according to the Profiles 4.3 of the GB/T 17657 - 1999 Test methods of evaluating the properties of wood-based panels and surface decorated wood-based panels. The hardness of the paint film of the finished floor board is determined according to the GB/T6739 - 1996 Determination of film hardness by pencil test. The density of the wood uncompressed is determined according to the GB 1933 - 91 Method for determination of the density of wood. The density of the floor board compressed is determined according to the Profiles 4.2 of the GB/T 17657- 1999 Test methods of evaluating the properties of wood-based panels and surface decorated wood-based panels. The abrasion resistance of the surface of the paint film of the floor board is determined according to the GB/T 15036.2-2001 Solid wood flooring-Examination and test methods.

## Claims

1. A manufacturing method for a surface-strengthened solid wood floor board wherein the density of it is 300 ∼ 580Kg/m³, the thickness of the reinforced surface is 1 ∼ 5mm, the hardness of a paint film on the reinforced surface according to the Standard GB/T6739-1996 is 2H ∼ 8H and overall moisture content of the profiles is 6 ∼ 9%, comprising the following steps:
( 1 ) Drying log profiles, the moisture content of the dried wood profiles being controlled within 7 ∼ 16%;
( 2 ) Compressing the log profiles by the hot press within 210°C-250°C, the pressing speed of the hot press being within 4mm/s ∼ 10mm/s;
( 3 ) Keeping warm the profiles obtained after the compression for 20-60 minutes by keeping the temperature of the hot press at the temperature of step (2) or 10°C-80°C. lower than the hot pressing temperature of step (2) and maintaining pressure;
( 4 ) Controlling the moisture content of the profiles within 6-9%;
( 5 ) Tonguing and grooving the profiles;
( 6 ) Surface sanding and finishing,

2. The manufacturing method for the surface strengthened solid wood floor board as claimed in claim 1, **characterized in that** during the said step of drying log profiles, moisture content of the dried wood profiles are controlled within 7-13%.

3. The manufacturing method for the surface stengthened solid wood floor board as claimed in claim 1, **characterized in that** surface of the wood profiles are polished after drying log profiles.

4. The manufacturing method for the surface stengthened solid wood floor board as claimed in claim 1, **characterized in that** the temperature of the hot press in step (2) is controlled within 230°C-250°C.

5. The manufacturing method for the surface stengthened solid wood floor board as claimed in claim 1, **characterized in that** the compression ratio of the log profiles in step (2) is within 15%-25%.

6. The manufacturing method for the surface stengthened solid wood floor board as claimed in claim 1, **characterized in that** the said compressed log profiles are kept warm for 20-40 minutes.

7. The manufacturing method for the surface stengthened solid wood floor board as claimed in claim 1, **characterized in that** the moisture content of the profiles in step (4) is controlled within 7-8%.

8. The manufacturing method for the surface stengthened solid wood floor board as claimed in claim 1, **characterized in that** controlling moisture content of the profiles within 6-9% in step (4) is achieved by the step of putting the profiles in the moisture control room, whose temperature is 40°C-65°C and relative humidity is 75%-95%.

## Patentansprüche

1. Herstellungsverfahren für einen oberflächenverstärkten Massivholzbodenbelag, wobei seine Dichte 300 - 580 kg/m³ ist, die Dicke der verstärkten Oberfläche 1 - 5 mm ist, die Härte eines Lackfilms auf der verstärkten Oberfläche gemäß dem Standard GB/T6739-1996 2H - 8H ist und der gesamte Feuchtigkeitsgehalt der Profile 6 - 9% ist, das die folgenden Schritte umfasst:
(1) Trocknen von Baumstammprofilen, wobei der Feuchtigkeitsgehalt der getrockneten Holzprofile innerhalb von 7 - 16% gesteuert wird;
(2) Komprimieren der Baumstammprofile durch die Heißpresse innerhalb von 210°C - 250°C, wobei die Pressgeschwindigkeit der Heißpresse innerhalb von 4 mm/s - 10 mm/s liegt;
(3) 20 - 30 Minuten Warmhalten der nach der Kompression erhaltenen Profile, indem die Temperatur der Heißpresse bei der Temperatur von Schritt (2) oder 10°C - 80°C niedriger als die Heißpresstemperatur von Schritt (2) gehalten wird und der Druck aufrecht erhalten wird;
(4) Steuern des Feuchtigkeitsgehalts der Profile innerhalb von 6 - 9%;
(5) Ausbilden von Nut und Feder in den Profilen;
(6) Schleifen und Endbearbeiten der Oberfläche.

2. Herstellungsverfahren für den oberflächenverstärkten Massivholzbodenbelag nach Anspruch 1, **dadurch gekennzeichnet, dass** der Feuchtigkeitsgehalt der getrockneten Holzprofile während des Schritts zum Trocknen von Baumstammprofilen innerhalb von 7 -13% gesteuert wird.

3. Herstellungsverfahren für einen oberflächenverstärkten Massivholzbodenbelag nach Anspruch 1, **dadurch gekennzeichnet, dass** die Oberfläche der Holzprofile nach dem Trocknen der Baumstammprofile poliert wird.

4. Herstellungsverfahren für einen oberflächenverstärkten Massivholzbodenbelag nach Anspruch 1, **dadurch gekennzeichnet, dass** die Temperatur der Heißpresse in Schritt (2) innerhalb von 230°C - 250°C gesteuert wird.

5. Herstellungsverfahren für einen oberflächenverstärkten Massivholzbodenbelag nach Anspruch 1, **dadurch gekennzeichnet, dass** das Kompressionsverhältnis der Baumstammprofile in Schritt (2) innerhalb von 15% - 25% liegt.

6. Herstellungsverfahren für einen oberflächenverstärkten Massivholzbodenbelag nach Anspruch 1, **dadurch gekennzeichnet, dass** die komprimierten Baumstammprofile 20 - 40 Minuten lang warm gehalten werden.

7. Herstellungsverfahren für einen oberflächenverstärkten Massivholzbodenbelag nach Anspruch 1, **dadurch gekennzeichnet, dass** der Feuchtigkeitsgehalt der Profile in Schritt (4) innerhalb von 7 - 8% gesteuert wird.

8. Herstellungsverfahren für einen oberflächenverstärkten Massivholzbodenbelag nach Anspruch 1, **dadurch gekennzeichnet, dass** das Steuern des Feuchtigkeitsgehalts der Profile innerhalb von 6 - 9% in Schritt (4) durch den Schritt des Legens der Profile in den Feuchtigkeitskontrollraum, dessen Temperatur 40°C - 65°C ist und dessen relative Feuchtigkeit 75% - 95% ist, erreicht wird.

## Revendications

1. Procédé de fabrication de plancher en bois massif renforcé en surface, dans lequel la densité de celui-ci est de 300 à 580 kg/m³, l'épaisseur de la surface renforcée est de 1 à 5 mm, la dureté d'un feuil de peinture sur la surface renforcée selon la Norme GB/T6739-1996 est de 2 H à 8 H et le taux global d'humidité des profilés est de 6 à 9 %, comportant les étapes suivantes :
(1) séchage de poutres profilées, le taux d'humidité des profilés en bois séchés étant maintenu dans un intervalle de 7 à 16 % ;
(2) compression des poutres profilées dans une presse à chaud à une température de 210°C à 250°C, la vitesse de compression étant de 4 mm/s à 10 mm/s ;
(3) maintien au chaud des profilés obtenus après la compression pendant 20 à 60 minutes en conservant la température de la presse à chaud à la température de l'étape (2) ou 10°C à 80°C au-dessous de la température de compression à chaud de l'étape (2) et en maintenant la pression ;
(4) régulation du taux d'humidité des profilés dans un intervalle de 6 à 9 % ;
(5) bouvetage et mortaisage des profilés ;
(6) ponçage et finissage.

2. Procédé de fabrication de plancher en bois massif renforcé en surface selon la revendication 1, **caractérisé en ce que**, pendant ladite étape de séchage de poutres profilées, le taux d'humidité des profilés en bois séchés est maintenu dans un intervalle de 7 à 13 %.

3. Procédé de fabrication de plancher en bois massif renforcé en surface selon la revendication 1, **caractérisé en ce que** la surface des profilés en bois est polie après le séchage des poutres profilées.

4. Procédé de fabrication de plancher en bois massif renforcé en surface selon la revendication 1, **caractérisé en ce que** la température de la presse à chaud lors de l'étape (2) est maintenue dans un intervalle de 230°C à 250°C.

5. Procédé de fabrication de plancher en bois massif renforcé en surface selon la revendication 1, **caractérisé en ce que** le taux de compression des poutres profilées lors de l'étape (2) se situe dans un intervalle de 15 % à 25 %.

6. Procédé de fabrication de plancher en bois massif renforcé en surface selon la revendication 1, **caractérisé en ce que** lesdites poutres profilées comprimées sont maintenues au chaud pendant 20 à 40 minutes.

7. Procédé de fabrication de plancher en bois massif renforcé en surface selon la revendication 1, **caractérisé en ce que** le taux d'humidité des profilés lors de l'étape (4) est maintenu dans un intervalle de 7 à 8 %.

8. Procédé de fabrication de plancher en bois massif renforcé en surface selon la revendication 1, **caractérisé en ce que** le maintien d'un taux d'humidité des profilés dans l'intervalle de 6 à 9 % lors de l'étape (4) est réalisé par l'opération consistant à mettre les profilés dans la salle de régulation d'humidité où la température est de 40°C à 65°C et l'humidité relative est de 75 % à 95 %.
